

## UNITED STATES PATENT OFFICE

2,475,672

## PROCESS FOR PRODUCING A TEXTILE FABRIC HAVING THE TWO SIDES THEREOF IN DIFFERING COLORS

Albert Mellor and Ralph James Mann, Spondon, near Derby, England, assignors, by mesne assignments, to Celanese Corporation of America, a corporation of Delaware.

No Drawing. Application September 14, 1944, Serial No. 554,149. In Great Britain September 24, 1943

4 Claims. (Cl. 8—15)

1

This invention relates to the production of coloured textile fabrics.

We have found that valuable textile fabrics can be obtained by applying a saponifying agent to a textile fabric consisting of or containing cellulose acetate or other cellulose ester fibres and causing saponification to take place, the conditions being such that saponification of the cellulose ester fibres is effected to a substantial degree on one side of the fabric while the cellulose ester fibres on the other side of the fabric remain unsaponified or are saponified to a considerably less degree. Such fabrics are very useful since by dyeing with suitable dyes they can readily be coloured so that the shade of one side differs from that of the other. For example, by dyeing a fabric saponified in this way with both a direct cotton dye and a cellulose ester dye it is possible to colour the two sides of the fabric in entirely different shades. Moreover, these valuable effects can be obtained upon fabrics of simple construction and without the necessity for weaving a fabric from two different kinds of fibres and arranging that fibres of one kind predominate on one side of the fabric and fibres of the other kind predominate upon the other side of the fabric. Thus the effects can be obtained on fabrics comprising cellulose ester fibre yarns which appear on both sides of the fabric. In the saponified fabrics individual yarns have portions visible on one side of the fabric which are saponified and portions visible on the other side which are unsaponified.

Most conveniently the saponifying agent is applied to one side of the fabric in the form of a preparation so thickened that it does not penetrate through to the opposite side of the fabric to any substantial extent. As thickening agents, various water-soluble gums can be employed, for example gum tragacanth. Such water-soluble thickening agents may be supplemented or replaced by water-insoluble inorganic thickeners, for example French chalk, fuller's earth, kaolin or like material of an absorbent character. These specific materials consist substantially of metal silicates.

It is very advantageous first to apply to the side of the material which has to remain substantially unsaponified a mechanical or chemical resist which prevents unwanted saponification on the side to which it is applied. For this purpose water-soluble gums, such as gum gatto, can be employed. Again, insoluble water repellent substances, for example fats or waxes, can be used. Further, the resist may comprise an acid, e. g.

2

a solid water-insoluble acid and particularly a higher fatty acid, for instance stearic acid or palmitic acid or other fatty acid containing at least 12 carbon atoms. These water-insoluble acids may, if desired, be used in conjunction with a water-repellent wax, for example paraffin wax.

We have further found that in the case of acid resists it is not essential to restrict the application of the acid to one side of the cellulose ester fabric. Extremely good results can be obtained, for instance, by applying a thickened saponifying medium to one side only of a fabric which has been uniformly impregnated with an acid substance. Though the acid substance is neutralised by the saponifying agent on the side of the material to which the latter is applied, it nevertheless serves to localise the action of the saponifying agent and to reduce substantially or prevent saponification of the fibres on the opposite side of the material. Higher fatty acids are very suitable for use as resists in this manner. They may, for instance, be applied to the material in the form of solutions in volatile organic liquids, e. g. volatile chlorinated hydrocarbons, and the volatile liquid removed by evaporation. Again, they may be applied to the material in the form of aqueous solutions of their ammonium salts and the material then heated so as to decompose the ammonium salt, drive off the ammonia and leave the fatty acid on the material. This latter is a particularly convenient way of utilising the higher fatty acids such as stearic or palmitic acid.

The saponifying agents or the resists or both may be applied to the fabric either locally or over the whole surface of the fabric. Again the saponification may be to different degrees as between different saponified portions of the fabric with corresponding differences in dye affinity. Thus the saponifying agent may be applied over the whole surface of the fabric and local removal of saponifying agent effected, for example by bringing the moist material into contact with a surface engraved in a pattern. In this way, for instance, fabrics can be obtained which, on dyeing with a suitable dye or mixture of dyes yield on the saponified side effects resembling the well known "batik" effects.

As saponifying agents, the alkali metal hydroxides and carbonates are especially useful. They can be applied to the material in the form of aqueous solutions, thickened for instance in the manner described above, and the desired saponification of one side of the fabric effected or completed by drying the material, for exam-

ple in hot air or on steam-heated cans. After application of the aqueous saponifying agent to the material, the latter may be allowed to remain in the moist state for a short time, for example 1-5 minutes, before drying. By suitably prolonging the period during which the material is allowed to remain in the moist state the required saponification can usually be obtained without drying the material; avoidance of drying has the advantage that the thickening agent is more readily washed from the material. After saponification has been effected any residual saponifying agent should be neutralised, for example by treatment with dilute hydrochloric acid or other aqueous acid. The fabric is then washed to free it from products of the saponification reaction and from the thickening agents and resists employed. The degree of saponification of individual filaments should be such as to impart affinity for direct cotton dyes.

The two sides of fabric saponified in the above manner can be dyed in a wide range of contrasting shades by dyeing the fabric on the one hand with a dye which has affinity for the cellulose ester but little or no affinity for cellulose and on the other hand with a dye which has affinity for cellulose but little or no affinity for unsaponified cellulose ester. The saponified material takes up the dye having affinity for cellulose. It may also take up the cellulose ester dye to a greater or less degree, depending on the extent to which the filaments have been saponified. The dye used for colouring the unsaponified cellulose ester is advantageously of the water-insoluble type applied in the form of an aqueous dispersion. The two types of dye may be applied to the material in separate operations or they may be applied in a single bath when compatible one with the other. Printing and other methods of applying dyes locally to the material may be employed if desired. Again, dischargeable colouring matters can be employed either for the saponified material or for the unsaponified material or both and the coloured materials subjected to a discharge printing operation. A very wide range of differentially coloured and patterned materials can thus be obtained.

If desired dyes or dye components capable of being fixed on the saponified portion of the material can be applied in conjunction with the saponifying agent thus effecting simultaneous saponification and colouring. Thus vat dyes in leuco form or as sulphuric esters of the leuco compounds, e. g. Soledon Jade Green XS or Indigosol O, can be included and subsequently converted to the parent vat dyes on the saponified portions of the material. Again enolic coupling components having affinity for cellulose, for example arylamides of 2:3-hydroxynaphthoic acid or other ortho-hydroxy-carboxylic acid, or arylamides of aceto-acetic acid or other beta-keto-carboxylic acid, can be included and subsequently developed to azo dyes on the material with diazo compounds; if desired diazo compounds in stabilised form can be used and applied together with the enolic coupling component.

The invention is illustrated by the following examples:

*Example I*

A cellulose acetate fabric of twill weave is secured, dried, and padded in an aqueous solution prepared with 50 to 75 grams per litre of stearic acid and sufficient ammonia to dissolve the latter. The padding is conducted so that the material

retains about 75% of the aqueous solution based on the weight of the fabric. The material is then dried. Alternatively the stearic acid can be applied as a 50 to 75 grams per litre solution in perchlorethylene and the material then dried. The material is then back-filled with a paste of the following composition:

200 grams 6% gum tragacanth, 20 grams caustic soda in 50 ccs. water, 35 grams French chalk.

The fabric is then allowed to hang in the air for 1-5 minutes, dried and the remaining alkali quickly neutralised by treatment with dilute hydrochloric acid. Finally, the fabric is thoroughly washed and then dyed in a single bath containing both a direct cotton dye and a water-insoluble dye having direct affinity for cellulose acetate.

The dyeing can be accomplished for instance 20 on the jigger in a bath containing 2 grams per litre of soap at 80° C. using the following mixture of dyes:

|                                                     | Per cent |
|-----------------------------------------------------|----------|
| 25 2:4 - dinitro-4'-amino-diphenylamine (10% paste) | 0.45     |
| 1 - amino - 4 - hydroxy - anthraquinone (10% paste) | 0.30     |
| Durazol Fast Yellow B 400 powder (I. C. I.)         | 0.5      |
| Durazol Fast Blue 4 G. 200 powder (I. C. I.)        | 1.0      |

The percentages of the dyes are based on the weight of the material. Again it can be accomplished at 80° C. in a 150:1 bath containing 1 gram per litre of sodium lauryl sulphate and 12 30 grams per litre of common salt using the following mixture of dyes:

|                                                                               | Per cent |
|-------------------------------------------------------------------------------|----------|
| 2:4 - dinitro-4'-amino-diphenylamine (10% paste)                              | 1.8      |
| 40 1 - amino - 4 - hydroxyanthraquinone (10% paste)                           | 1.50     |
| 1 - methylamino - 4 - (beta - hydroxyethyl-amino) - anthraquinone (10% paste) | 0.1      |
| Durazol Fast Yellow B 400 powder (I. C. I.)                                   | 3.0      |
| 45 Chlorazol Brown MS (I. C. I.)                                              | 0.5      |
| Chlorantine Fast Blue GLL 200 powder C. A. C.)                                | 0.1      |

The percentages of the dyes are based on the weight of the material. The side to which the saponifying agent has been applied is coloured a chocolate shade and the other side a yellowish brown shade.

*Example II*

55 A fabric of the kind referred to in Example I is scoured and dried and the face is filled with an aqueous solution of gum gatto containing 30 grams of gum per litre. The material is then dried and is then back-filled with the alkaline saponifying paste referred to in Example I. Subsequent treatment of the fabric is also effected as in Example I.

Having described our invention, what we desire to secure by Letters Patent is:

1. In a process for the production of a textile fabric having the two sides thereof colored in different colors by a dyeing process, the steps which comprise substantially completely impregnating a textile fabric comprising fibers of an organic acid ester of cellulose with a solid water-insoluble fatty acid containing at least 12 carbon atoms, applying to the one side of the fabric a solution of a saponifying agent so thickened that it fails to penetrate through to the opposite side, permitting the saponifying agent to saponify the

organic acid ester of cellulose fibers on the side to which it is applied and thereafter dyeing the fabric with a dye having an affinity for the organic acid ester of cellulose fibers but not for the saponified fibers and with a dye having an affinity for the saponified fibers but not for the organic acid ester of cellulose fibers.

2. In a process for the production of a textile fabric having the two sides thereof colored in different colors by a dyeing process, the steps which comprise substantially completely impregnating a textile fabric comprising fibers of cellulose acetate with a solid water-insoluble fatty acid containing at least 12 carbon atoms, applying to the one side of the fabric a solution of a saponifying agent so thickened that it fails to penetrate through to the opposite side, permitting the saponifying agent to saponify the cellulose acetate fibers on the side to which it is supplied and thereafter dyeing the fabric with a dye having an affinity for the cellulose acetate fibers but not for the saponified fibers and with a dye having an affinity for the saponified fibers but not for the cellulose acetate fibers.

3. In a process for the production of a textile fabric having the two sides thereof colored in different colors by a dyeing process, the steps which comprise substantially completely impregnating a textile fabric comprising fibers of cellulose acetate with stearic acid, applying to the one side of the fabric a solution of a saponifying agent so thickened that it fails to penetrate through to the opposite side, permitting the saponifying agent to saponify the cellulose acetate fibers on the side to which it is applied and thereafter dyeing the fabric with a dye having an affinity for the cellulose acetate fibers but not for the saponified fibers and with a dye having

an affinity for the saponified fibers but not for the cellulose acetate fibers.

4. In a process for the production of a textile fabric having the two sides thereof colored in different colors by a dyeing process, the steps which comprise substantially completely impregnating a textile fabric comprising fibers of cellulose acetate with palmitic acid, applying to the one side of the fabric a solution of a saponifying agent so thickened that it fails to penetrate through to the opposite side, permitting the saponifying agent to saponify the cellulose acetate fibers on the side to which it is applied and thereafter dyeing the fabric with a dye having an affinity for the cellulose acetate fibers but not for the saponified fibers and with a dye having an affinity for the saponified fibers but not for the cellulose acetate fibers.

ALBERT MELLOR.  
RALPH JAMES MANN.

#### REFERENCES CITED

The following references are of record in the file of this patent:

#### UNITED STATES PATENTS

| Number    | Name         | Date          |
|-----------|--------------|---------------|
| 646,379   | Tagliani     | Mar. 27, 1900 |
| 1,266,955 | Kniffler     | May 21, 1913  |
| 2,020,698 | Platt        | Nov. 12, 1935 |
| 2,068,770 | Schwarzchild | Jan. 26, 1937 |
| 2,145,364 | Moncrieff    | Jan. 31, 1939 |
| 2,248,048 | Allan        | July 8, 1941  |

#### FOREIGN PATENTS

| Number  | Country       | Date          |
|---------|---------------|---------------|
| 346,544 | Great Britain | Apr. 16, 1931 |

**Certificate of Correction**

Patent No. 2,475,672

July 12, 1949

**ALBERT MELLOR ET AL.**

It is hereby certified that errors appear in the printed specification of the above numbered patent requiring correction as follows:

Column 3, lines 71 and 72, Example I, for the word "secured" read *scoured*; column 4, line 26, for "(10" read *(10%*; column 5, lines 19 and 20, for "supplied" read *applied*; and that the said Letters Patent should be read with these corrections therein that the same may conform to the record of the case in the Patent Office.

Signed and sealed this 10th day of January, A. D. 1950.

[~~SEAL~~]

**THOMAS F. MURPHY,**  
*Assistant Commissioner of Patents.*